

Dec. 6, 1932.

W. H. WOOD

1,890,242

ELECTROLYTIC DIAPHRAGM

Filed June 23, 1927



Fig. 1



Fig. 2



Fig. 3



Fig. 4



Fig. 5

Fig. 6



Fig. 8



Fig. 7



Fig. 9

William H. Wood  
Inventor  
by Smith and Freeman  
Attorneys

## UNITED STATES PATENT OFFICE

WILLIAM H. WOOD, OF SOUTH EUCLID, OHIO

## ELECTROLYTIC DIAPHRAGM

Application filed June 23, 1927. Serial No. 200,866.

This invention relates to the porous diaphragms employed in certain electrolytical operations to separate different liquids or electrodes from each other while permitting the ready migration of ions, and the particular device to which my invention is chiefly directed is known in the art as a storage battery separator although many features of my invention are susceptible of wider use. It is important in devices of this nature that the porosity be high, the texture uniform, pinholes and other openings being avoided, and a substantial amount of physical strength exhibited together with at least a substantial degree of resistance to the chemical action of the electrolyte. Separators made solely of simple substances like cloth, wood, earthenware, perforated insulation and the like have been found unsatisfactory for various reasons which have resulted in attempts to make separators of a complex construction, employing a frame of some kind of supporting and strengthening material such for example as vulcanized rubber, having wicks or capillary inclusions supported therein. The objects of the present invention is the provision of a new, simplified, and improved process whereby the manufacture of such composite separators or diaphragms is facilitated, and whereby an increased portion of the fibers or wick-forming materials are run transversely of the separator from one face to the other thereof, and whereby those wicks or capillaries are arranged in substantially uniform and regular manner over the surface of the same.

In the drawing accompanying and forming a part of my application I have illustrated in a diagrammatic way a series of steps constituting a part of my improved process of producing such separators together with a specimen separator produced thereby. It will be understood that several of the actual steps are not susceptible of ready illustration, so that no attempt is made to illustrate all the manipulations and procedures, but only to portray sufficient to enable those skilled in the art to form successfully the invention in question; and that certain of the steps I have actually shown can be

eliminated or modified without departure from the scope of my invention.

Fig. 1 is a vertical longitudinal section of a mixing and rolling apparatus and illustrates steps of mixing and rolling which constitute a part of my invention; Fig. 2 is a perspective view of a small section of the sheet produced thereby; Fig. 3 is a magnified view of a small portion of said sheet; Fig. 4 is a top plan view of another rolling machine illustrating an optional process for increasing the regularity of location of the wicks or fibers; Fig. 5 is a perspective view of a section of the sheet produced thereby; Fig. 6 is a magnified view of a small section of that sheet; Fig. 7 is a perspective view of a block illustrating the mode of combining together a plurality of the before-mentioned sheets and subsequently severing the same to form separators; Fig. 8 is a perspective view of one of the complete separators so made; and Fig. 9 is an enlarged microscopic view of a portion of said separator.

The matrix material which I employ is hereafter referred to as rubber, but by that term I do not limit myself strictly to the sap of the so-called rubber tree, but intend to include other substances having the herein-essential properties of rubber, namely elasticity, vulcanizability, resistance to electrolyte-corrosion, and high resistance to electric currents. As a wick-forming or capillary material I preferably employ organized keratin in fibrous form as set forth in my Patents Nos. 1,405,703 and 1,502,455, preferably in the form of mammalian hair from which the scales have been loosened or removed by appropriate chemical treatment, as by the action of lime or sodium sulfite. However, it is equally within the purview of the present invention to employ untreated hair, or birds-feathers, cotton, hemp or other previous cellulose strands, flax, disintegrated plant stems, or other capillary substance which occurs in fibrous form, the choice being determined partly by financial considerations and partly by the chemical nature of the electrolyte.

The fibrous material is preferably chopped into such lengths as can be readily mixed

with the rubber and as will produce relatively straight sections of wick material. This chopping is not imperative, since some substances like hair can be employed without such comminution and some substances like 5 wool-waste, cotton-lint, etc. can be secured in this ready-made form. This wick-material is mixed with the rubber-like material in any suitable manner as by the automatic, 10 power-driven mixing machine illustrated at 1 in Fig. 1, from which it passes in a regulated manner, the item of regulation being here implied by the auger screw feed 2, through an extruding nozzle 3 which delivers the mass in the form of a ribbon to a 15 series of rolls 4, 5, 6, 7, 8, be the same more or less in number, by which the material is reduced to the form of a thin, elongated sheet 10. It is desirable that the length of at least the greater part of these fibrous 20 materials be greater than the thickness of the sheet, and necessary that it be greater than the thickness of the separator which is to be made and I preferably employ about the largest amount of such fibrous material as will produce a homogeneous and bubble-free mixture in combination with the matrix substance. Inasmuch as the permissible limits of composition are extremely wide I do not 25 deem it necessary to afford any strict proportions, although an example of a possible proportion is three parts by weight of rubber to one part by weight of fibrous material. The larger the proportion of fiber, the larger the 30 porosity of the resulting separator, while the large the proportion of rubber the greater is the strength of the same. The choice of 35 composition necessarily rests upon the use to which the device is to be put. It will be found that the mixture thus made is an extremely 40 sticky and unpleasant material to handle, but is entirely within the ability of standard rubber machines and processes, it being assumed that the rollers are made of the proper materials, maintained at proper 45 temperatures, and applied with proper dusting and anti-sticking substances.

A cut of the sheet 10 is shown at Fig. 2, and a small portion taken from the point 11 thereof is shown under the microscope in Fig. 3, where it will be seen that the fibers 12 run somewhat criss-cross but always within the plane of the sheet and prevailingly in one direction due to the rolling process.

It is possible with perfectly satisfactory 55 results to jump from this point immediately to the step illustrated in Fig. 7 but it is preferable for certain uses at this point to interpose a further step designed to bring the fibrous material more nearly parallel to a given direction, and thereby increase the porosity of the separator for a given stiffness. To do this I pass the sheet 10 through a further series of rolls illustrated in Fig. 4 which 60 are preferably arranged directly in sequence

to the first described rolls, the same comprising smooth faced cylindrical rolls 15 and circumferentially corrugated rolls 16 arranged in alternation to any desired number. The tendency of the corrugations is to arrange the fibers lengthwise of the sheet by squeezing them into little bundles while the effect of the smooth surfaced rolls is to flatten the surface of the sheet without at the same time restoring the irregular arrangement of the fibers, with the result that most of the fibers ultimately become arranged lengthwise of the sheet while still remaining wholly within the top and bottom surface thereof. 70 75 80

The sheet produced as above described is severed into rectangular segments 10 or 17 as the case may be which are laid one upon the other as shown in Fig. 7 until a pile 18 is produced having the cross sectional shape and size of the separator or other diaphragm desired, and the whole vulcanized. Care is exercised that the surfaces of the sheets are sufficiently clean to insure their adhering together into a unitary mass, after which slices are removed from said pile transverse to the planes of said sheets as shown at 19 in Fig. 7. In case of any predominant location of the fibers in a given direction as shown in Figs. 5 and 6 the sheets are so laid as to 95 maintain such direction uniform in all the sheets, and the plane of slicing is transverse to that direction so that the majority of those fibers traverse the resulting separator from side to side. 100

In some cases the mere act of rolling illustrated in Fig. 1 produces a predominant lengthwise trend of the fibrous material so that the particular step illustrated in Fig. 4 for emphasizing the lengthwise arrangement is not necessary. Indeed it will be seen that the mere act of producing a sheet which is thinner than the length of the majority of the fibers exercises a degree of selection by preventing a vertical position of said fibers and increases the proportion of fibers which traverse the resulting separator from side to side even though no other selective action existed. The mere action of rolling lengthwise, particularly by successive steps with the consequent gradual increase of speed (since it is obvious that the rolls 8 must rotate faster than the rolls 4 to transmit a given weight of material per unit of time) necessarily helps to arrange the fibers lengthwise. The further production of strands by the use of corrugated rolls carries the selection slightly further. 110 115 120

It is immaterial so far as concerns my invention whether the vulcanizing be effected all at once and the individual separators severed after its completion, or whether the separators be given a further heat treatment after they are severed from the block. The particular mode and extent of vulcanizing or hardening the material is also immaterial to 125 130

the present invention. As heretofore stated, the fibers and the matrix substance can be made of various materials; the apparatus illustrated is chosen only as one example of what can be done, and I do not limit myself except as recited in my several claims which I desire may be construed each independently of limitations contained in other claims.

Having thus described my invention what I claim is:

- 10 1. The process of making a porous diaphragm for electrolytic use which contains the steps of mixing indiscriminately together a plastic matrix substance and a fibrous per-  
15 vious substance, rolling such mixture repeat-  
edly in the same direction, superposing the sheets thereby produced to form a pile with the grain of the majority of said sheets par-  
20 allel, causing said sheets to adhere together,  
and slicing such pile transversely of the grain.
2. The process of making a porous dia-  
phragm for electrolytic use which contains the steps of mixing intimately together a  
25 plastic matrix substance and a fibrous per-  
vious substance, forming said mixture into sheets, forming said sheets alternately into corrugated form and smooth form until the fibers are arranged prevailingly in one direc-  
30 tion, collecting the sheets into a pile, harden-  
ing said pile, and slicing said pile transverse-  
ly of said sheets and of the prevailing direc-  
tion of said fibers.

In testimony whereof I hereunto affix my  
35 signature.

WILLIAM H. WOOD.

40

45

50

55

50